# EUROPEAN PATENT SPECIFICATION

(11) **EP 1 563 042 B1**
(45) Date of publication and mention of the grant of the patent: **11.03.2009**
(21) Application number: 03811402.1
(22) Date of filing: 12.11.2003
(51) Int. Cl.: C10L 1/18, C10L 10/04

(54) **Method for Manufacturing a Fuel Additive**
Verfahren zur Herstellung eines Kraftstoffadditivs
Procédé de Fabrication d'un Additif pour Carburant

(30) Priority: 20.11.2002 FI 20022069
(43) Date of publication of application: 17.08.2005
(73) Proprietor: Forchem Oy, 26101 Rauma (FI)
(72) Inventor: FREDRIKSON, Martti, FIN-26100 Rauma (FI); AHONEN, Heikki, FIN-37720 Ritvala (FI)
(74) Representative: Laitinen, Pauli Sakari
(86) International application number: PCT/FI2003/000856
(87) International publication number: WO 2004/046282

(56) References cited:
- EP-A1- 0 635 558
- US-A- 5 952 518
- US-A- 5 968 211
- DATABASE CA [Online] KOICHIRO UCHITA ET AL.: 'Gas oil compositions with improved lubricity properties', XP002980013 Retrieved from STN Database accession no. 129:56338 & JP 10 130 666 A 19 May 1998

## Description

The present invention relates to a method for manufacturing a fuel additive. The invention particularly relates to a lubricating additive, which is highly suitable for use as an additive in diesel engines.

The continual increase in price of fuels, particularly fuels for combustion engines, and the tightening of environmental legislation have led to numerous proposals for improvement and actual improvements in both engines and fuels.

In automotive engines, engines based on the diesel cycles are gaining ground over petrol engines, due to the greater thermal efficiency of diesel engines. In addition to the existing efficiency based on a high compression ratio, engine operation has been further improved with better injection of the fuel into the combustion chamber.

While environmental requirements have led to a great reduction of sulphur in these fuels, polyaromatic and other cyclic compounds, which as such have excellent lubricant properties in high-pressure fuel-injection devices, have also been removed along with the sulphur.

Fatty acids have been proven to be good additives to fuels, especially diesel fuels. However, fatty acids have the well-known drawback that they either crystallize easily, or else that stearic acid and arachid acid can easily crystallize out of them, in other words, fatty acids as such are not suitable for very cold conditions. Even the esters of these acids easily crystallize out of, for example, olive oil as fats.

US patent 8,129,772 discloses a fuel additive, which is manufactured from saturated fatty acids and oligomeric fatty acids, in which tertiary amines are used as crystallization inhibitors. The patent particularly emphasizes that mixtures of different saturated fatty acids are not used, but no grounds are given for this.

US patent 5,578,090 discloses a fuel and a fuel additive, characterized in being formed from the esters of fatty acids, some of which are glycerine esters and some triglycerides.

WO 94/17160 discloses a fuel additive, which is formed of fatty acids, which are esterified with alcohols containing one or more carbons.

EP 826765 discloses a corresponding diesel-fuel additive, which is a partial ester of a fatty acid and a polyol, for example, an ester of glycerine and monocarboxylic acid, and which is added in 75 - 200 ppm to middle runnings.

US 3,765,850 discloses a fuel additive, which is obtained by allowing dicarboxylic acid to react with polyamides.

US patent 6,156,082 discloses that it is not advantageous for a fuel additive to be esterified, because lubricity will suffer. Instead, it presents partial esterification with diethylene glycolin and an organic acid anhydride, which gives good lubricity results.

US patent 6,194,361 discloses that a usable lubricant can be obtained from the distilled fatty acids of tall oil, by allowing the fatty acids of tall oil to react with diethanolamine, and by allowing the fatty acid to react with aminoethyl piperazidine. This compounds is used, for among other purposes, lubricating oil-drilling boreholes, both with oil and as a water emulsion.

US patent 6,197,731 discloses that a suitable two-stroke engine lubricant is obtained by esterifying polyols with polycarboxylic acids.

JP 08092581 discloses how the -OH group of castor oil is esterified with a saturated monovalent fatty acid, thus creating a lubricant that functions at an extremely low temperature.

US patent 6,086,645 discloses how a fuel additive can be advantageously created by manufacturing carboxylic acid amines for this purpose, from oleic acid and/or linolenic acid.

US patent 5,882,364 discloses a corresponding fuel additive, which is formed of esters of an unsaturated fatty acid and a polyvalent alcohol, two different grades of which are mixed together in the same mixture.

US patent 6,203,584 discloses a fuel additive, which is formed of the esters of polyvalent carboxylic acid and a polyoxyamine and of a mixture, which acts together with them, of carboxylic acid and a polyvalent alcohol.

US patent 5,997,593 discloses a fuel additive, which is formed of the reaction product of carboxylic acid and an amine, in which the said amine is guanidine, amineguanidine, urea, or thiourea.

US patent 6,051,039 discloses a diesel fuel additive, which is obtained from an amine of dicarboxylic acid, which is an amine derivative of succinic acid or phthalic acid and a mixture of them and of an NR₃ amine, in which R contains 6-24 carbon. This mixture is added to diesel fuel in a concentration of at least 1000 ppm.

US patent 5,556,972 discloses how fats can be fractioned by crystallizing the stearin ester fraction of out a fatty-acid fraction in two stages and removing the said stearin fat fraction by filtration. The hardening point of the fat is thus reduced. The process is carried out using counter-flow crystallization and thus reduces the solidification point of margarine, for example.

US patent 5,952,518 discloses a method, by means of which fatty acids with a high melting point can be removed from other fatty acids. In this case, an emulsifying agent is used as an aid, the mixture is cooled and the saturated fatty acids are removed from the mixture by crystallization. A polyvalent alcohol and esters of a fatty acid are used as the emulsifier. The fatty acids are hydrolyzed rapeseed oil or soya oil.

As is stated in many patents, the fatty acids of tall oil act well as lubricants in combustion engines, as do their alcohol esters with alcohols and the amines of fatty acids. However, fatty acids as such would be the best lubricants. Saturated fatty acids and their derivatives are said to be particularly good as lubricants.

Throughout history, particularly stearic acids and their salts have been used as excellent lubricants.

According to patent application FI20011214, a fatty acid composition is cold-treated in a heat exchanger, in which the saturated fatty acids, such as stearic acid and arachid acid separate onto a cold surface and this fraction is esterified and aminated and combined with a mother liquor fraction after this. Using this procedure, the amount of acids in the mother liquor that precipitate at low temperatures is reduced to about 1/4 - 1/5. Further, in this cold crystallization, many other fatty acids remain trapped amount the needle-like crystals that form, so that the content of stearic acid in the fraction being esterified and aminated will have only quadrupled, compared to the original content.

The present invention is intended to further improve the process, by means of which fuel of the type described in the aforementioned patent application is manufactured. This is achieved in the manner stated as characterized in the accompanying Claims.

According to the present invention, at least part of the solvent used in the crystallization is a solvent that is used in a later stage in the esterification of the crystal phase, which solvent is removed from the mother liquor by distillation. Thus it has been observed that, in the presence of an alcohol, a branched alcohol, or a similar solvent, the crystal phase becomes different, and not needle-like, as it does without the solvent. The crystal phase can then be easily separated from the mother liquor by centrifuging.

One extremely advantageous alcohol is 2-propanol, in the presence of which plate-like, easily sedimented and separated crystals are formed from, for example, stearic acid, when other fatty acids are present. The same can be achieved using, for instance, propyleneglycol-n-butyl ether (Dowanol PnB), which has a boiling point of 170°C and a freezing point of - 75°C. Correspondingly, it is possible to use propyleneglycol-n-propyl ether, which has a boiling point of 149°C and a freezing point of -80°C (Dowanol PnP). Further, it is possible to advantageously use, for example, 1-methoxy-2-propanol (Dowanol PM glycolether).

All of the compounds referred to as examples have in common a branched hydrocarbon chain, with an -OH group at the end of the chain. With the aid of this -OH group, the product can be esterified with fatty acids.

According to the present invention, stearic acid and arachid acid are crystallized out of tall oil in the presence of an auxiliary solvent, which auxiliary solvent can be an alcohol or ether, which can as such be esterified later, or a solvent that does not interfere with further use, or a mixture of these. Surprisingly, it has been observed that typical diesel oil or light fuel oil is also such an auxiliary solvent, which improves the separation of the crystals, even if it is not esterified in the following stage. However, the best auxiliary solvent appears to be isopropanol. Therefore, according to this invention, saturated fatty acids, which separate when cold (< +5°C) in the presence of an auxiliary solvent, are separated by crystallization, are esterified preferably using branched alcohols or ethers containing -OH groups, these being distilled out of the mother liquor of the crystallization and mixed with the said mother liquor and the esterified fatty-acid mixture, and used an additive and lubricant in an engine fuel, preferably diesel fuel. This can also be used as a lubricant in normal petrol, which is required as the engines of petrol-powered automobiles begin to use direct injection of fuel into a pressurized cylinder, as is presently done in diesel engines.

According to observations that have been made, it is preferable to use products containing more than one -OH group for esterification, and particularly preferable for them to be branched, or at least iso-alcohols, or iso-esters of an alcohol. If these are used as auxiliary agents in crystallization, they need not be removed at all from the crystal phase, the same products that are distilled out of the mother liquor being instead added to the said crystal phase prior to esterification. The use of more than one mixture containing -OH groups is advantageous, because this reduces the solidification point of the mixture and naturally also reduces the cloud point of the fuel, in which the said additive is mixed.

Isopropanol is clearly the best auxiliary solvent for aiding the crystallization described above and the separation of the crystals. This alcohol has a boiling point of 82.5°C and can easily be separated by distillation and easily esterified with fatty acids with the aid of an acid catalyst. In abrasion tests (HFRR +60°C, ISO 12156-1) that were carried out, it appeared that solely a fatty-acid mixture, such as that obtained from the vacuum distillation of tall oil (TOFA-2), was the best lubricant in an abrasion test in a mixture of diesel oil, the crystallization mother liquor described above being used as the fatty-acid mixture.

Further, it is possible to advantageously use a DBE solvent (dimethyl glutarate + dimethyl adipate - dimethyl succinate), which achieves complex esterification with the said crystal phase, as an aid in the aforementioned esterification process. DBE is a commercial solvent, which is obtained as a byproduct of the manufacture of polyesters. The reaction of this DBE and fatty acids resulted in a viscous liquid, while methanol was released from the reaction.

The accompanying figure shows a diagram of one example of process equipment according to the invention. According to the figure, the product (fatty acid = FA), is brought to a reservoir 1 together with a solvent or solvent mixture, is cooled, for example, in a heat exchanger 2, and is given a sufficient delay to crystallize, while being slowly mixed in a vessel 3, after which the mixture is led to a separating device 4. The separating device can be a filter or a centrifuge, from which the crystal phase is led through a heater 7 to an esterification vessel 5, to which a catalyst, for example phenol sulphonic acid or toluene sulphonic acid, is also led. The 'mother liquor' obtained from the separator 4 is led to distillation, from which the solvent or solvents are led back to the reservoir 1, the basic product of the distillation being combined with the esterified fatty acids obtained from the vessel 5 to create the finished product.

Results: Auxiliary agent always totals 500 ppm = Fatty acid + its esters in diesel oil without additives.

| Product | Cloud point | HFRR wear |
|---|---|---|
| Diesel oil without additives | -27.3°C | 619 µm |
| Commercial winter-grade diesel | -42°C | 410 µm |
| Fatty acid mother liquor | -24.3°C | 265 µm |
| Fatty acid 500 ppm as such | -28.0°C | |
| TOFA mother liquor 50 % + 50 % PnB | | |
| + DBE esters | -35.4°C | 347 µm |
| TOFA mother liquor 50 % + DBE ester | | |
| (crystal phase) 50 % | -34.5°C | 294 µm |
| TOFA mother liquor + isopropyl ester | | |
| 25 % + FA diethanol amide 25 % | -42°C | 317 µm |

The cloud-point measurements are not entirely indisputable, but are indicative. The accuracy of the measurement appears to be ±2°C. From the above table, it can be seen that using solely tall oil fatty acids at a content of 500 ppm will achieve good lubricity properties. However, they are not suitable for conditions with temperatures below -27°C.

In the above descriptions, the esterification and possible amination were carried out as a crystal phase on the separated part of the fatty acids while the auxiliary solvents were distilled out of the mother liquor. FA = fatty acid. It is obvious that isopropanol will distill very completely out of the fatty-acid mixture, but that, for example, PnP and PnB will distill poorly, because PnB has a boiling point of 170°C and PnP 149°. However, as both of them have a cloud point in the order of -80°C, it is advantageous to leave small amounts of them among the fatty acids.

## Claims

1. A method for manufacturing fatty-acid compounds for use as a lubricant additive to fuel, in which stearic acid and arachid acid are separated from a fatty-acid mixture by cooling, are esterified, the esterified mixture thus obtained being mixed again with the part of the original fatty-acid mixture from which the fatty acids have been separated, the necessary amount of this latter mixture being mixed with fuel as a lubricant, **characterized in that** the fatty-acid mixture is separated in the presence of a solvent or solvent mixture containing alcohol groups, that the solvent or solvent mixture is used to esterify the removed fatty acids, that the said solvents are removed from the mother liquor, and that the esterified fractions are combined with the residue of the mother liquor and used as an additive in fuel.

2. A method according to Claim 1, **characterized in that** esters containing alcohols or groups of alcohols, the boiling point of which is less than +180°C, are used as the solvents.

3. A method according to Claim 1, **characterized in that** the solvents are selected from the group: isopropanol, tert. butanol, n-butoxy propanol, propylene glycol n-propyl ester.

4. A method according to Claim 1, **characterized in that** at least part of the product separated by crystallization is esterified by complex esterification with the methyl esters of bivalent organic acids.

5. A method according to Claim 1, **characterized in that** the fatty-acid phase is separated in the presence of organic solvents containing alcohol groups, in the temperature range 0 - 5°C, and that the separation is carried out by filtering, sedimentation, or centrifuging.

6. A method according to any of the above Claims, **characterized in that** the solvent containing alcohol groups is used in an amount corresponding to 10 - 50 % of the amount of the fatty acid.

7. A method according to any of the above claims, **characterized in that** at least 20 % of the solvent is isopropanol.

## Patentansprüche

1. Verfahren zur Herstellung von Fettsäureverbindungen zur Verwendung als Schmiermittelzusatz von Brennstoff, wobei Stearinsäure und Arachidsäure durch Abkühlung aus einem Fettsäuregemisch getrennt werden, verestert werden, wobei das **dadurch** erhaltene veresterte Gemisch wieder mit demjenigen Teil des ursprünglichen Fettsäuregemisches vermischt wird, aus dem die Fettsäuren getrennt worden sind, wobei die erforderliche Menge dieses letzteren Gemisches als Schmiermittel mit Brennstoff vermischt wird, **dadurch gekennzeichnet, dass** das Fettsäuregemisch in der Gegenwart eines Lösungsmittels oder einer Alkoholgruppen enthaltenden Lösungsmittelgemisches getrennt wird, dass das Lösungsmittel oder Lösungsmittelgemisch zur Veresterung der entfernten Fettsäuren verwendet wird, dass besagte Lösungsmittel aus der Mutterlauge entfernt werden, und dass die veresterten Fraktionen mit dem Rückstand der Mutterlauge kombiniert werden und als Zusatz im Brennstoff verwendet werden.

2. Verfahren nach Anspruch 1, **dadurch gekennzeichnet, dass** die Alkohole oder Alkoholgruppen enthaltenden Ester, deren Siedepunkt unter +180°C liegt, als Lösungsmittel verwendet werden.

3. Verfahren nach Anspruch 1, **dadurch gekennzeichnet, dass** die Lösungsmittel aus folgender Gruppe ausgewählt sind: Isopropanol, tert-Butanol, n-Butoxy-propanol, Propylenglykol-n-propylester.

4. Verfahren nach Anspruch 1, **dadurch gekennzeichnet, dass** zumindest Teil des durch Kristallisation getrennten Produkts durch komplexe Veresterung mit den Methylestern von zweiwertigen organischen Säuren verestert wird.

5. Verfahren nach Anspruch 1, **dadurch gekennzeichnet, dass** die Fettsäurephase in der Gegenwart von organischen, Alkoholgruppen enthaltenden Lösungsmitteln im Temperaturbereich 0-5°C getrennt wird und dass die Trennung durch Filterung, Sedimentation oder Zentrifugieren erfolgt.

6. Verfahren nach einem der obigen Ansprüche, **dadurch gekennzeichnet, dass** das das Alkoholgruppen enthaltende Lösungsmittel in einer Menge eingesetzt wird, die 10-50 der Menge der Fettsäure entspricht.

7. Verfahren nach einem der obigen Ansprüche, **dadurch gekennzeichnet, dass** zumindest 20 % des Lösungsmittels Isopropanol sind.

## Revendications

1. Procédé pour fabriquer des composés acides gras pour être utilisés comme additif lubrifiant pour carburant, dans lequel l'acide stéarique et l'acide arachide sont séparés par refroidissement, sont estérifiés, le mélange estérifié ainsi obtenu étant mélangé de nouveau avec la partie du mélange orignal d'acide gras à partir de laquelle les acides gras avaient été séparés, la quantité nécessaire de ce mélange étant mélangée avec le carburant comme lubrifiant, **caractérisé en ce que** le mélange d'acide gras est séparé en présence d'un solvant ou d'un mélange de solvant contenant des groupes alcooliques, que le solvant ou le mélange de solvant est utilisé pour estérifier les acides gras enlevés, que lesdits solvants sont enlevés de la liqueur mère, et que les fractions estérifiées sont combinées avec le reste de la liqueur mère et utilisées comme additifs dans un carburant.

2. Procédé selon la revendication 1, **caractérisé en ce que** les esters contenant des alcools ou des groupes alcooliques, dont le point d'ébullition est moins de +180 °C, sont utilisés comme solvants.

3. Procédé selon la revendication 1, **caractérisé en ce que** les solvants sont sélectionnés dans le groupe de : isopropanol, alcool butylique tertiaire, n-butoxy propanol, éther monopropylique du propylène glycol.

4. Procédé selon la revendication 1, **caractérisé en ce qu'**une partie au moins du produit séparé par cristallisation est estérifiée par une estérification complexe avec les éthers méthyliques d'acides organiques bivalents.

5. Procédé selon la revendication 1, **caractérisé en ce que** la phase d'acide gras est séparée en présence de solvants organiques contenant des groupes alcooliques, dans une gamme de température de 0 à 5 °C, et que la séparation est effectuée par filtrage, sédimentation ou centrifugation.

6. Procédé selon l'une quelconque des revendications ci-dessus, **caractérisé en ce que** le solvant contenant des groupes alcooliques est utilisé dans une quantité correspondant à 10 à 50 pour cent de la quantité de l'acide gras.

7. Procédé selon l'une quelconque des revendications ci-dessus, **caractérisé en ce que** 20 pour cent au moins du solvant est de l'alcool isopropylique.
